

## ANTI-CORROSION COMPOSITIONS

Jean Suprin, Notre-Dame-de-Gravenchon, and Francis Soldano, Les Aigalades-Marseille, France, assignors to Esso Standard Societe Anonyme Francaise, Paris, France, a body corporate

No Drawing. Filed Jan. 18, 1956, Ser. No. 559,793

Claims priority, application France Mar. 19, 1955

2 Claims. (Cl. 252—33.4)

The present invention relates to corrosion inhibiting compositions, and particularly relates to compositions comprising hydrocarbon oils and minor proportions of the reaction products of C<sub>8</sub>—C<sub>24</sub> fatty acids and ethylene diamine or diethylene triamine.

The additive compounds used in the compositions of the present invention are obtained by reaction between fatty acids and di- or tri-alkyl amines.

Thus a reaction between oleic acid and ethylene diamine is carried out at temperatures of about 140°—160° C. to obtain oleylamidoethylamine as represented by the equation:



Oleylamidoethylamine may be further reacted with a fatty acid, e.g. oleic acid, to form the corresponding salt, e.g. oleylamidoethylamine mono-oleate,



which may in turn be dehydrated to form dioleylamidoethane, C<sub>17</sub>H<sub>33</sub>.CO.NH.C<sub>2</sub>H<sub>4</sub>.NH.CO.C<sub>17</sub>H<sub>33</sub>.

In preparing the above types of compounds any saturated or unsaturated C<sub>8</sub>—C<sub>24</sub> fatty acid may be used, which may contain one or more hydroxyl groups. The preferred fatty acids include lauric, palmitic, stearic, oleic, linoleic, ricinoleic, oleomargaric, erucic, behenic arachidic or lignoceric acids.

Corresponding compounds may be prepared using diethylene tri-amine. The additive compounds obtained from reaction between the fatty acid and di- or tri-ethylamines may be incorporated in hydrocarbon oils in amounts between 0.01% and 10% by weight based on the total composition.

The hydrocarbon oils in which the additive compounds are incorporated may be any hydrocarbon, e.g. a petroleum fraction, in which they are soluble. They are preferably mineral lubricating oils, which may be used to prevent the rusting of inaccessible systems, or to prevent the rusting of metal parts during processing or storage. Compositions of the present invention comprising lubricating oils may advantageously be employed in equipment which requires lubrication in addition to protection from corrosion, such as in circulating oil and hydraulic systems, bearings, instruments or internal combustion engines.

In another type of application the corrosion inhibiting compounds of the present invention may be incorporated in volatile solvent-type hydrocarbons such as gasolines, kerosines, white-spirits, or gas-oils. Such compositions generally contain also a film-forming material such as wax, resin, or petrolatum. When such compositions are applied to a metal surface, the volatile solvent evaporates in a short time, and leaves a thin film which inhibit rusting of the metal.

A particular advantage of the compositions of the present invention is that they are ashless, e.g. do not form metallic deposits, when used in internal combustion en-

gines, or after being burnt off metal surfaces during annealing or other operations.

The present invention therefore comprises anti-corrosion compositions comprising a hydrocarbon oil and a minor proportion of the reaction product of a C<sub>8</sub>—C<sub>24</sub> fatty acid and ethylene diamine or diethylene triamine.

Having now described the invention in broad terms, reference may be made to the following example.

## EXAMPLE I

Tests were carried out on plates of hot-rolled bright steel covered with anti-rust compositions according to the invention. Two compositions were used in this series of test, both being based on naphthenic mineral oil of viscosity 155 cs. at 100° F. Sample "I" consisted of the base oil containing 5% of dioleylamido ethane, and sample "II" consisted of the base oil containing 5% of oleylamidoethylamine oleate.

The steel plates were cleaned by sandblasting, covered with the compositions under test, and stabilized for 16 hours in a box under ambient conditions. The covered plates were then transferred to a humidity cabinet, where they were spaced apart in an upright position, and exposed to continual condensation of water vapour at a temperature of 100° F. The efficacy of the anti-rust compositions was taken as the minimum time in hours taken by a plate to show the first signs of rust.

The results of this test are shown in Table I wherein the test samples are compared with the straight base oil.

Table I

|    | Anti-rust liquid                                       | Time taken for rust to appear, hours |
|----|--------------------------------------------------------|--------------------------------------|
| 35 | Base Oil                                               | 24                                   |
|    | Sample "I" (Base oil +5% dioleylamido ethane)          | 1,700                                |
|    | Sample "II" (Base oil +5% oleylamidoethylamine oleate) | 1,300                                |

It will be seen from the test results shown in Table I that compositions of the present invention were very effective in delaying the onset of rust on steel plates, compared with straight mineral oil.

A further aspect of the present invention is that a well-defined anti-corrosive synergistic effect is obtained when the additive compounds of the present invention are incorporated in hydrocarbon oils together with minor proportions of oil-soluble naphthenates or sulphonates of alkaline or alkaline-earth metals. The preferred sulphonates are those with a molecular weight between 300 and 600, and may conveniently be derived from petroleum "mahogany" acids, or from other sources, e.g. from the polypropyl benzene hydrocarbons obtained as a heavy alkylate during the manufacture of dodecyl benzene. Thus if from 0.01% to 5%, preferably 0.1% to 3% of the said sulphonates or naphthenates are incorporated in the said hydrocarbon oils, much loss of the fatty acid/amine reaction products are required to give effective anti-corrosion properties. Thus from 0.01% to 3% of the additive product may be sufficient. This effect is illustrated by Example II below.

## EXAMPLE II

65 Eight compositions numbered III to X comprising a mineral naphthenic oil of viscosity 155 cs. at 100° F. from 1.5% to 2.3% of sodium sulphonate of molecular weight 500, and various proportions, usually 0.8% of fatty acid/amine reaction products according to the present invention were used to cover bright steel plates as in Example I, and after stabilization for 16 hours were placed in a humidity cabinet, where the corrosion evalua-

tion of the various compositions evaluated as before. The results are shown in Table II below.

2. An anti-corrosion composition consisting of a naphthenic mineral oil having a viscosity of about 155 cs. at

Table II  
ANTI-RUST COMPOSITION

|                                       | Control | III    | IV    | V    | VI   | VII   | VIII  | IX    | X     |
|---------------------------------------|---------|--------|-------|------|------|-------|-------|-------|-------|
| Mineral Base Oil, percent             | 97.7    | 97.1   | 97.1  | 97.1 | 97.1 | 97.1  | 97.1  | 97.1  | 97.1  |
| Sod. sulphonate (MW 500)              | 2.3     | 2.1    | 2.1   | 2.1  | 2.1  | 2.1   | 2.1   | 2.1   | 2.1   |
| Oleylamidoethylamine                  |         | 0.8    |       |      |      |       |       |       |       |
| Stearylamidoethylamine                |         |        | 0.8   |      |      |       |       |       |       |
| Laurylamidoethylamine                 |         |        |       | 0.8  |      |       |       |       |       |
| Ricinoleylethylamine                  |         |        |       |      | 0.8  |       |       |       |       |
| Dioleylamidoethane                    |         |        |       |      |      | 0.8   |       |       |       |
| Oleyl-2 imidazole                     |         |        |       |      |      |       | 0.8   |       |       |
| Ethylene diamine dioleate             |         |        |       |      |      |       |       | 0.8   |       |
| Time taken for rust to appear (hours) | 90      | >1,580 | 1,200 | 850  | 600  | 1,580 | 1,500 | 1,460 | 1,100 |

It will be noted from the results shown in Table II, that much less of the fatty acid/amine reaction product is required to endow anti-corrosion properties when incorporated in hydrocarbon oils with sulphonates, than when the products are contained in the oils alone.

It is to be understood that in addition to the rust-inhibitor additives of the present invention there may be added to the hydrocarbon oil base stocks other agents such as dyes, pour depressors, heat thickened fatty oils, sulphurised fatty oils, organo metallic compounds, metallic or other soaps, sludge dispersants, anti-oxidants, thickeners, viscosity index improvers, other corrosion inhibitors, oiliness agents, resins, olefin polymers, or volatilized fatty oils, fats, mineral oils, waxes, graphite or zinc oxide.

What we claim is:

1. An anti-corrosion composition comprising: a major amount of a hydrocarbon oil; 0.1 to 3 wt. percent of an alkali metal petroleum sulfonate having a molecular weight in the range of 300 to 600; and 0.01 to 3 wt. percent of the dehydrated amide reaction product of 2 moles of a  $C_8-C_{24}$  fatty acid and one mole of ethylene diamine.

100° F., about 2.1 wt. percent of a sodium petroleum sulfonate having an average molecular weight of about 500, and about 0.8 wt. percent dioleylamidoethane.

#### References Cited in the file of this patent

#### UNITED STATES PATENTS

|    |            |                  |                |
|----|------------|------------------|----------------|
| 25 | Re. 23,227 | Blair et al.     | May 9, 1950    |
|    | 2,481,585  | Freeman          | Sept. 13, 1949 |
|    | 2,493,483  | Francis et al.   | Jan. 3, 1950   |
|    | 2,598,213  | Blair et al.     | May 27, 1952   |
| 30 | 2,640,029  | Blair et al.     | May 26, 1953   |
|    | 2,646,399  | Hughes           | July 21, 1953  |
|    | 2,720,490  | Oxford           | Oct. 11, 1955  |
|    | 2,763,614  | Cantrell et al.  | Sept. 18, 1956 |
|    | 2,791,495  | Rudel et al.     | May 7, 1957    |
| 35 | 2,798,045  | Buck et al.      | July 2, 1957   |
|    | 2,828,259  | Wirtel et al.    | Mar. 25, 1958  |
|    | 2,882,227  | Lindberg         | Apr. 14, 1959  |
|    | 2,888,399  | Wirtel et al.    | May 26, 1959   |
|    | 2,902,447  | Gunderson et al. | Sept. 1, 1959  |